

Oct. 4, 1938.

T. L. SHEPHERD

2,131,983

ELASTIC YARN AND METHOD OF MAKING IT

Filed Feb. 23, 1937



T. L. Shepherd  
invention

By: Glascock Downing Subd  
Atty's

## UNITED STATES PATENT OFFICE

2,131,983

## ELASTIC YARN AND METHOD OF MAKING IT

Thomas Lewis Shepherd, London, England

Application February 23, 1937, Serial No. 127,257  
In Great Britain February 28, 1936

9 Claims. (Cl. 117—57)

This invention relates to rubber processes and products in which rubber is manufactured in thread or filament form and also to processes and products involved in or resulting in fabrics such as woven, knitted or lace work, formed from or incorporating such threads or filaments.

The word "thread" will be hereinafter used to cover thread or filament.

Rubber may be manufactured in such form according to one method by extruding latex or other coagulable dispersions of rubber or rubber-like materials with or without other ingredients such as vulcanizers, accelerators, reinforcing fillers, anti-oxidants and stabilizers.

In British patent specifications Nos. 447,972, 448,098, 449,314 and 449,462 and British patent applications Nos. 10,448/35, 18,200/35 and 30,481/35, I describe processes in which there is mixed with the latex or latex mixture for extrusion purposes, or with a liquid coagulant for the latex, when such is used or in which there is otherwise intimately mixed with the rubber, various extensibility-reducing agents, such as glue, gelatine and similar proteins, casein, albumen, natural and synthetic resins and gums which are water soluble, cellulose esters and ethers (e. g. methyl cellulose), and inorganic (e. g. sodium silicate) or organic substances (e. g. sugar) which dissolve in water to give solutions which are miscible with the latex without coagulation. It is not intended to be implied that all such substances will be advantageous from every aspect, for example, as is well known, copper salts greatly accelerate the rate of perishing of rubber from the *Hevea brasiliensis*, so that in selecting the extensibility-reducing agent regard must be had to the possibility of such other effects. When the latex mixture is extruded or otherwise formed into thread by processes in-

cluding coagulating the rubber, and is dried, a relatively inextensible thread is produced, which may be woven or otherwise manipulated without the difficulties associated with extensible threads. Relatively inextensible threads can also be made according to British patent application No. 30,481/35, according to which an extensibility-reducing agent may be incorporated with rubber by masticating the extensibility-reducing agent with rubber in a compounding mill, or mixing it with a rubber dough in a colloid mill, the threads being formed as desired, for instance by cutting a sheet of the rubber or the like mixture.

Elastic yarns not of this relatively inextensible character when covered with fine cotton or silk

spun thread suffer from serious defects, the principal ones being:—

(1) In the winding process the cores have to be subjected to a very severe stretch, in some instances approaching the figure of 370 per cent., for otherwise the winding flyers, which cover the core at high speed, would be ineffective. As a result, the core cannot later retract to its more or less normal length because to a great extent the textile covering prevents it. There is also a tendency for the tension to be not or not quite even. When incorporated into fabric, the weaving brings out this uneven tension and the cloth is puckered in parts, a fault which cannot be permanently remedied.

(2) The textile winding has an insufficient grip on the core and slips and this shows itself when the covered core is subjected either in the weaving, knitting, or lacating machine or in the fabric to tension, a tension which it is the normal function of the thread or fabric to resist. The textile covering should extend and contract with the core but owing to the aforementioned slip this does not always happen and it is found that in some places the textile winding or covering becomes displaced in its relation to the core. In such places the fabric again shows a permanent pucker.

(3) The cost of cotton or silk covering is very high, as only very fine spun yarns can be utilized. The high cost of covering material brings the price of the complete fabric or article very often to a prohibitive level, and the cheaper artificial silk filaments cannot be used as they are considered too slippery.

The object of the invention is to provide processes for the manufacture of improved yarns, and another object of the invention is to overcome the above disadvantages.

According to the present invention a relatively inextensible thread, as before referred to, is used, and enables satisfactory winding to take place at a much lower stretch, whilst the presence of extensibility-reducing agent modifies the surface of the thread by rendering the surface plastic so that the possibility of slipping is much reduced, both in the case of textile threads and of artificial silk threads because these threads form grooves in the plastic core thread.

The invention will be pointed out in the accompanying claims.

In the drawing there is diagrammatically shown a core thread *a* and a helically wound covering thread *b*, the latter being shown as if removed

from the lefthand side of the figure to show permanent grooves c.

By the employment of the thread of the character referred to, the winding operation is facilitated in that the requisite conditions for winding can be attained with a stretch of 15 per cent. or lower. The tendency for the tension to be not or not quite even is minimized or entirely lost, on account of the small stretch.

10 In order to attain the advantages mentioned the threads which are applied must not be wound loosely. The tightness which is required will vary with different cases but no tightness above that which is normal with threads not of the 15 character referred to is generally necessary for obtaining the advantages to a good degree.

The braiding or winding is applied by the usual braiding or winding machines.

20 The subsequent removal of the extensibility-reducing agent allows my core to take on a more pronounced and deeper groove for the winding to rest in and any traces of extensibility-reducing agent which may remain in my core have the action of still more firmly anchoring the winding 25 to the core.

The grooves are slightly more pronounced when the core is wound in a non-vulcanized condition but the grooving also takes place when winding a vulcanized core.

30 If, owing to rough handling or accidents, the textile covering becomes damaged or broken, it may therefore be prevented from unwinding or becoming separated from the core; it may be arranged that such damage can hardly be detected with the naked eye, when the nature of 35 the core is such that the winding will in the dyeing process have assumed the same shade as the rubber core underneath.

It is now possible to utilize for winding or lac- 40 ing material even a filament hitherto considered slippery, such as artificial silk as made from viscose, cellulose acetate, cuprammonium and other materials. This filament need not be spun from staple fibre (although it may be if desired) 45 as is the case with cotton or real silk from fibres but may be extruded. I may use such filaments for winding singly or in multiples and these multiples may either be in a twisted condition or lie parallel. Apart from reducing the cost of the 50 covering material considerably, this artificial silk winding renders it possible to weave or knit or lace a multitude of new fabrics heretofore unknown and I can now produce elastic fabrics and articles with a new pleasing and beautiful appear- 55 ance and new effects can be obtained by careful pre-selected incorporation of the artificial silk covered elastic thread into other materials, producing either uniformly dyed finished fabrics or cross-dyed fabrics.

60 The relatively inextensible thread may be caused to hold itself extended during the application of the covering. For instance, when gelatine is the extensibility-reducing agent, the thread may be wound after the core has been 65 given under steam a predetermined amount of stretch, varying as desired from 1 per cent. to as much as 600 per cent. or more and dried before covering, which leaves it, owing to its nature, in this stretched condition.

70 The covering with textile matter may also be applied to the core when it is in a non-, semi-, or fully vulcanized condition.

After the application of heat, steam, or boiling fluids, when they are applied for getting rid of 75 the extensibility-reducing agent, the covered core

will then try to assume its old shorter pre-stretched shape, but it is to a large extent prevented from doing so by the surrounding textile covering.

However, as the stretch may be pre-determined, the subsequent tension set up in the rubber core by the covering can be arranged to be even and in the weaving, knitting or lacing no puckering takes place.

The invention may be used in conjunction with 10 the processes described or claimed in British specifications Nos. 423,997, 440,256, 441,002, 441,124, 441,465, 442,931, 442,935, 442,936, 442,937, 443,284, 443,914, 447,972, 448,098 and 449,462 and British application No. 5,085/36. 15

If desired in addition to the textile coverings hitherto referred to a filament of gelatine or of other soluble substance, may be applied over the textile covering. Such soluble filament may be caused to adhere firmly to the textile covered 20 thread by treating the resulting yarn with solvent in suitable form for the soluble thread. For instance, treatment of a gelatine helical winding with steam will result in firm adhesion. By this means the extensibility of the yarn is practically 25 eliminated.

The gelatine or like winding or the like may be removed by dissolving it away after the fabric has been made.

In a modification a band or tape of gelatine 30 or the like instead of a filament may be used over the textile covering.

A gelatine or like coating may be applied to the textile or artificial silk covering by passing the covered yarn through a solution of gelatine and 35 allowing the coating to harden or set.

Reference is also made in a preceding paragraph to British specification No. 449,462, in which it is envisaged to render glue or gelatine insoluble by means of formaldehyde when it is used as an extensibility-reducing agent, and after the thread has been formed. The same process, which results in a thread of permanently reduced extensibility, may be used in conjunction with the present invention, as well as analogous processes whereby other extensibility-reducing agents may be rendered insoluble in water.

I claim:

1. A method of manufacturing a yarn which consists in incorporating in a normally elastic 50 core thread a quantity of extensibility reducing agent sufficient to produce a relatively inextensible and plastic thread, and embedding a textile winding in said thread to form permanent grooves therein whereby slipping of the textile winding 55 is prevented.

2. A method of manufacturing a yarn which consists in incorporating in a normally elastic core thread a quantity of extensibility reducing agent sufficient to produce a relatively inextensible and plastic thread, stretching the thread while moist, drying the stretched thread and embedding a textile winding in said dried and stretched thread to form permanent grooves 60 therein whereby slipping of the textile winding 65 is prevented.

3. A method of manufacturing a yarn which consists in incorporating in a normally elastic core thread a quantity of extensibility reducing agent sufficient to produce a relatively inextensible and plastic thread, embedding a textile winding in said thread to form permanent grooves 70 therein, and covering the said textile winding with a soluble filament.

4. A method of manufacturing a yarn which

consists in incorporating in a normally elastic core thread a quantity of extensibility reducing agent sufficient to produce a relatively inextensible and plastic thread, embedding a textile winding in said thread to form permanent grooves therein, covering the said textile winding with gelatine.

5. A method of manufacturing a fabric which consists in incorporating in a normally elastic core thread a quantity of extensibility reducing agent sufficient to produce a relatively inextensible and plastic thread, embedding a textile winding in said thread to form permanent grooves therein whereby slipping of the textile winding 10 is prevented, incorporating said thread into a fabric, and removing the extensibility reducing 15 agent from the fabric.

6. A method of manufacturing a yarn which consists in incorporating in a normally elastic core thread a quantity of extensibility reducing agent sufficient to produce a relatively inextensible and plastic thread, embedding a textile winding in said thread to form permanent grooves therein whereby slipping of the textile winding 20 is prevented and treating the thread to render 25

the extensibility reducing agent partially insoluble to control the ultimate elasticity thereof.

7. A yarn comprising a core thread containing sufficient extensibility reducing agent to render the thread relatively inextensible and having permanent grooves and a textile winding embedded therein.

8. The method of manufacturing a fabric which consists in incorporating in a normally elastic core thread a quantity of extensibility reducing agent sufficient to produce a relatively inextensible and plastic thread, embedding a textile winding in said thread to form permanent grooves therein whereby slipping of the textile winding is prevented, incorporating said thread 15 into a fabric, treating the fabric to render the extensibility reducing agent partially insoluble to control the ultimate elasticity of the threads and removing the soluble extensibility reducing agent 20 from the fabric.

9. A method as claimed in claim 5 in which the extensibility reducing agent is removed by boiling in a bath containing a dye.

THOMAS LEWIS SHEPHERD.

25